

July 15, 1941.

P. ROBINSON ET AL

2,249,091

PROCESS FOR THE MANUFACTURE OF ELECTROLYTIC DEVICES

Filed June 15, 1937



BY

INVENTORS  
PRESTON ROBINSON &  
MATHEW NAZEWESKI  
*Dotay, Cole & Garner*  
ATTORNEYS

## UNITED STATES PATENT OFFICE

2,249,091

PROCESS FOR THE MANUFACTURE OF  
ELECTROLYTIC DEVICES

Preston Robinson, Williamstown, and Mathew Nazzewski, North Adams, Mass., assignors to Sprague Specialties Company, North Adams, Mass., a corporation of Massachusetts

Application June 15, 1937, Serial No. 148,398

1 Claim. (Cl. 154—2)

The present invention relates to electrolytic devices and more particularly to improvements in the construction of electrolytic condensers.

In various types of electrolytic devices, for instance, electrolytic condensers, a liquid and air-tight sealing of the device is of primary importance. Not only is this required to forestall the spilling of the electrolyte but also to prevent the salt dissolved in the electrolyte from creeping through leaks which may occur in the joints of such devices, a phenomenon which is characteristic of all electrolytic apparatus and which is due to the salt separating out of the solution. In fact, creepage of the electrolyte frequently takes place through joints which are seemingly impermeable to the liquid electrolyte. In view of the above and because of the importance of preventing contamination of the electrolyte by impurities which may enter through such leaks, the requirement of perfect sealing of such devices is evident.

The main difficulty in obtaining a liquid and air tight seal in electrolytic condensers and similar devices is due to the fact that outside electrical connection has to be made with the electrode or electrodes within the device and the joints between such connection and the sealing member, unless very expensive constructions are used, are likely to develop leaks.

For example, in a widely used construction for electrolytic condensers, a plug of soft rubber or similar resilient gasket material is provided through which passes a so-called electrode-riser, which serves for the support and electrical connection of the electrode.

To obtain a tight fit between the riser and the plug, a hole which is slightly smaller than that of the riser is provided in the plug. While this together with the crimping of the plug gives a substantially tight joint, still such a construction frequently permits a certain amount of creepage and loss of the electrolyte during the operation of the condenser and therefore is not a satisfactory solution of the problem.

The object of the present invention is to overcome the above difficulty and to provide an always reliable and permanently tight fit between the sealing plug and the electrode-riser passing through same.

In accordance with the invention, the plug is made of vulcanized rubber and after having been provided with a bore which is considerably smaller than one which would permit the electrode-riser to pass through same, is subjected to a swelling process, which temporarily causes ex-

pansion of the bore, thus permitting the riser to be passed through same. However, after the swelling liquid has evaporated, the bore tends to close up to its original diameter, thereby constantly exerting a very high pressure on the electrode-riser and providing between the plug and the riser for a very tight fit of permanent character.

Referring to the drawing which forms part of 10 the specification:

Figure 1 is a sectional elevation of an electrolytic condenser embodying the invention;

Fig. 2 is a perspective view of that end of the condenser of Fig. 1 which carries the plug of 15 the invention;

Fig. 3 is a sectional side-elevation of the condenser portion of Fig. 2;

Fig. 4 is an enlarged schematic drawing indicating the principle of the invention, and showing the rubber plug before and after its swelling. 20

Referring to the drawing, the condenser shown therein comprises a cylindrical metallic container 10, which preferably constitutes its cathode and which may be either of film-forming or non-film-forming metal. The container 10 is provided with a reduced tubular extension 12, threaded at 20 and extending into a further reduced tubular portion 21.

The anode assembly 28 as shown consists of 30 a corrugated thin foil 29 of aluminum or other film-forming metal, having the shape of an accordion pleating, which is suitably secured, for example by means of welding or by rivets, to an anode riser 30. The riser 30 consists of a 35 straight rod of rectangular or cylindrical shape and projects with its end 34 beyond the container portion 21. The anode riser 30 may be of aluminum or of other, preferably film forming, metal.

40 The top of the container is provided with a crowned metal cap 16, which fits into the container end 13. A vent gasket 14 of suitable material, for example of wax-impregnated cloth, is interposed between the container 10 and the cap 16.

45 The free edge of the cap 16, with the gasket 14 interposed, is crimped over a rim provided on the container 10.

Interposed between the container 10 and the anode assembly 28 is an insulator, for instance, 50 a thin hard rubber cylinder 32 provided with perforations 33, to prevent the anode foil 29 from contacting with the container 10.

The threads 20 are adapted to receive a nut (not shown) by means of which the condenser 55 may be attached to a suitable base.

The extension 21 has preferably the same inside diameter as the extension 12, so that the two form a common bore 22, the wall thickness of the extension 21 is however preferably much less than that of the extension 12.

Placed in the bore 22 is a tightly fitting plug 25 preferably of semi-hard vulcanized rubber through which passes the anode-riser 30.

In accordance with the invention the vulcanized rubber plug 25 is provided with a bore the cross-section of which is considerably less than that of the anode-riser. For example, if a round anode-riser is used having a diameter of .125 inch, the diameter of the hole should be about .060 to .070 inch.

We have found that if such a plug of vulcanized rubber is put into a solvent of the type of chloro-benzene, benzene, gasoline, dibutylamine, ether, and the like, the rubber swells and occupies a volume which is considerably in excess of its original volume, whereby the relative amounts of swelling depend on the solvent, the highest swelling being obtainable with chloro-benzene and benzene. It should be noted that such swelling takes place primarily at the surface of the rubber and that generally the greater portion of the rubber remains unchanged.

We have furthermore found that if a vulcanized rubber stopper is perforated with a fine clean-cut hole and the rubber is put into a solvent of the above type, the swelling takes place in such a manner that instead of the fine hole being blocked up by the swelling of the rubber as would be expected, the hole is caused to actually enlarge in diameter. What apparently takes place is that the increased volume of the swelled rubber pushes out the ends of the hole.

If now a metal rod such as the riser 30 is forced into the stopper, so that it makes a fairly tight fit in the enlarged hole of the swelled stopper, after the solvent has been allowed to evaporate, the rubber tends to revert to its original form, and thus exerts a considerable pressure on the metal rod. In this way a much tighter joint is obtained than if the rubber stopper were originally perforated to a diameter through which the rod can be forced without pre-swelling the stopper.

Applicants have found furthermore that the joint so obtained between the riser and stopper remains perfectly tight under all operating conditions.

Since water has the tendency to "wet" the surface of rubber, and since the majority of electrolytes used in wet electrolytic condensers contain water to a greater or lesser extent, it is preferable to add to the solvent used to swell up the rubber, a water-repellent agent. Such a water-repellent agent may be aluminum oleate or similar compounds which are soluble in the swelling agent.

For example if the anode riser, as stated, has a diameter of .125 inch, the stopper 25 is perforated by drilling therethrough a hole with a drill between #50 and #60 (diameters .070 inch to .040 inch). To obtain the desired results it is essential that the hole be absolutely clean-cut.

The perforated stopper is then placed into a suitable solvent, for example benzene—to which

a water-repellent agent, such as aluminum oleate, may be added in a quantity of  $\frac{1}{2}\%$  to 2% by weight—and left therein for a time period of several hours, the exact time depending primarily on the grade of rubber, the dimensions of the stopper and the hole drilled, and on the solvent. The hole will open to an extent that the riser can be pushed therethrough with comparative ease and without any tearing of the stopper. Thereafter the solvent is caused to evaporate from the plug. The evaporation may be carried on at room temperature or may be accelerated by placing the assembly in a heated air blast.

When the evaporation of the solvent has been completed, the plug 25, with the anode riser passing through the same, is inserted into the sleeve portion 21; the plug 25 should preferably be of such a length as to extend on both sides of the neck portion 21. Proper sealing between the plug 25 and the neck 21 may be obtained by a fluting operation such as described in the U. S. Patent No. 1,996,982 to Robert C. Sprague et al.

The electrolytes used in the condensers comprise as a rule, salts, acids, or alkalies and a solvent. Preferably, a combination of a weak acid and a salt is used, for instance, an electrolyte comprising borax and boric acid or ammonium borate and boric acid. However, various other acids and salts either alone or in combination give good results. For instance, phosphoric acid, citric acid, tartaric acid, and/or their salts are also suitable for electrolytes, whereby the salts do not need to be those of the acid used.

The viscosity of the electrolyte may range from that of water at 100° C. to that of a paste.

The invention is also of great utility when the electrical outside connection is made by means of comparatively small diameter wires, instead of rods as above described. To get good results blank and single strand (solid) wires should be used.

While we have described our invention with specific examples and in specific applications, it should be well understood that we do not wish to be limited thereto, but desire the appended claim to be construed as broadly as permissible in view of the prior art.

What we claim is:

In the manufacture of electrical condensers comprising a metal container, an electrode disposed in said container, and a terminal member secured to said electrode and protruding from an opening of said container, the method of providing an hermetically tight seal between said member and the container comprising the steps, providing in a flexible vulcanized rubber member a hole which is smaller in cross-section than the terminal member, swelling the rubber member in a volatile rubber solvent containing 0.5% to 2% by weight of aluminum oleate to increase by at least a factor of 2 the cross-section of said hole, disposing the terminal in the hole so enlarged, evaporating the solvent from the rubber member, disposing the rubber member in the opening of said container and crimping said container about said member.

PRESTON ROBINSON.  
MATTHEW NAZEWESKI.